

# UNITED STATES PATENT OFFICE.

KARL FARKAS, OF NEW YORK, N. Y., ASSIGNOR OF ONE-HALF TO GUY V. WILLIAMS,  
OF NEW YORK, N. Y.

## METALLIC FILAMENTS FOR INCANDESCENT ELECTRIC LAMPS.

1,008,807.

Specification of Letters Patent. Patented Nov. 14, 1911.

No Drawing.

Application filed August 9, 1909. Serial No. 511,998.

To all whom it may concern:

Be it known that I, KARL FARKAS, a citizen of the Kingdom of Hungary, and a resident of New York, in the county and State of New York, have invented certain new and useful Improvements in Metallic Filaments for Incandescent Electric Lamps, of which the following is a specification.

This invention has reference to a novel process of producing so called metallic filaments for incandescent electric lamps.

It pertains particularly to improvements in the production of metallic filaments prepared by pressure from fine powder of a highly refractory chemical element with glutinous substances in the well known manner, which substances act as binding materials. Such chemical elements adapted for this purpose are for instance, tungsten, molybdenum, osmium, chromium or ruthenium, etc. The metallic filaments thus prepared contain carbonaceous material because the glutinous substances are of organic origin. During the process of producing such filaments the glutinous substance is decomposed by heat and carbon set free which then forms part of the filament. Carbon, as is well known, consumes about three times the electric current to become incandescent as the pure highly refractory chemical element of which the filament is essentially composed. Therefore the finished filament pressed out of fine powder of such highly refractory chemical element should be entirely free from carbon.

I have discovered that metallic filaments prepared with glutinous organic binders may be freed entirely from carbon by embedding them in metallic oxides preferably the oxides of the earthy metals which must be in form of fine powder, heating them therein to a high temperature and finally heating them preferably to a higher temperature in the presence of oxygen gas. These filaments are embedded in a mixture of aluminum oxid and cerium oxid or they may be embedded in a mixture of aluminum oxid, magnesium oxid, and cerium oxid. During the process of heating, the glutinous substance is carbonized and decomposed and forms carbon *in statu nascendi* which, however, owing to the presence of the above oxides does not act on the highly refractory element of the filament but acts on the oxides.

The proportions in which the oxides are

employed are substantially as follows: About 90% of aluminum oxid is mixed with about 10% of cerium oxid or about 70% of aluminum oxid is mixed with about about 20% of magnesium oxid and about 10% of cerium 60 oxid. When the filaments have been embedded in the mixture of metal oxides, the box containing them is evacuated and then gradually heated up to about 1500° F. When this temperature has been reached 65 oxygen is introduced into the box from a reservoir in which the oxygen is preferably under some pressure. The quantity of oxygen introduced is measured on the barometer tube which indicates the vacuum. So 70 much of oxygen is introduced that the mercury in the barometer tube sinks about 1½ inches. The filaments are now further heated in the atmosphere of oxygen and the temperature is increased to about 2200° F. 75 During this time all carbonaceous material from the binder and all carbon resulting therefrom is combusted leaving a pure metallic filament of homogeneous structure and then the oxygen begins to oxidize slightly 80 the surface of the pure metallic filament producing thereon an exceedingly fine coating of oxid of the highly refractory elementary substance of which the filament is composed. When such filament is embodied in a lamp 85 the fine coating of oxid is rendered incandescent together with the entire filament.

The heating of the filaments in the vacuum furnace in an atmosphere of oxygen transforms completely any trace of carbonaceous material and carbon into carbon dioxide and further tends to oxidize or combust any other impurity which might mechanically adhere to the filaments. Thus the filament prepared according to the above 95 process is entirely free from carbon and on the surface of same a very fine coating of oxid is produced during the last stage of this process.

I claim as my invention:

1. The process of producing metallic filaments for incandescent electric lamps consisting in embedding shaped filaments of a highly refractory chemical element containing a glutinous organic binder in a mixture of metallic oxides, heating same under exclusion of the air to a high temperature, and then continuing the heating in the presence of oxygen.

2. The process of producing metallic fila-

100

90

95

105

110

- ments for incandescent electric lamps consisting in embedding shaped filaments of a highly refractory chemical element containing a glutinous organic binder in fine powder of oxids of the earthy metals, heating same under exclusion of the air to a high temperature, and continuing the heating up to a higher temperature in the presence of oxygen.
5. The process of producing metallic filaments for incandescent electric lamps consisting in embedding shaped tungsten filaments containing a glutinous organic binder in a mixture of metallic oxids, heating same *in vacuo* to a high temperature, and then continuing the heating to a higher temperature in the presence of some oxygen.
10. 3. The process of producing metallic filaments for incandescent electric lamps consisting in embedding shaped tungsten filaments containing a glutinous organic binder in a mixture of metallic oxids, heating same *in vacuo* to a high temperature, and then continuing the heating to a higher temperature in the presence of some oxygen.
15. 4. The process of producing metallic filaments for incandescent electric lamps consisting in embedding shaped tungsten filaments containing an organic binder in aluminum oxid mixed with some cerium oxid, heating same *in vacuo* to a high temperature, and continuing the heating to a higher temperature in the presence of oxygen.
20. 5. The process of producing metallic filaments for incandescent electric lamps consisting in embedding shaped tungsten filaments containing an organic binder in aluminum oxid mixed with some cerium oxid, heating same *in vacuo* to a high temperature, and then heating same in an atmosphere of oxygen up to a temperature of about 2200° F.
25. 6. The process of producing metallic filaments for incandescent electric lamps consisting in preparing by pressure filaments from fine powder of a highly refractory chemical element and a glutinous organic binder, embedding said filaments in aluminum oxid mixed with some cerium oxid, heating same *in vacuo* to a temperature of about 1500° F. and then heating same in an atmosphere of oxygen up to a temperature of about 2200° F.
7. The process of purifying metallic filaments containing carbon consisting in heating same *in vacuo* to a temperature of about 1500° F. and then heating same in an attenuated atmosphere of oxygen up to a temperature of about 2,200° F.
- Signed at New York, N. Y., this 7th day of August, 1909.

KARL FARKAS.

Witnesses:

LUDWIG K. BOHM,  
GUY V. WILLIAMS.